

May 11, 1926.

1,583,891

C. P. MADSEN

PROCESS FOR THE ELECTRODEPOSITION OF METALS

Original Filed Sept. 19, 1918



Patented May 11, 1926.

1,583,891

# UNITED STATES PATENT OFFICE.

CHARLES P. MADSEN, OF NEW YORK, N. Y., ASSIGNOR TO MADSENELL CORPORATION, OF NEW YORK, N. Y., A CORPORATION OF NEW YORK.

## PROCESS FOR THE ELECTRODEPOSITION OF METALS.

Application filed September 19, 1918, Serial No. 254,793. Renewed October 8, 1925.

My present invention relates to processes for the electrodeposition of metals from aqueous solutions as protective coatings or upon cathodes from which they are subsequently to be removed as final or intermediate articles of manufacture, especially as applied to metals such as nickel, iron, cobalt, etc.

Up to the present time very little or no success has been achieved in the production of deposits of such metals of any considerable thickness wherein the deposits are regular, homogeneous, smooth and malleable. Thus, in the production of nickel deposits 10 as hitherto practiced the deposits are not malleable and internal stresses are developed such that the deposit cracks or curls from its support on exceeding a thickness of 0.002-0.003 inch. By extreme care in controlling the conditions of the bath, practicable only in laboratory work, deposits as thick as 0.004 inch have occasionally been made; even then, however, the results have not been dependable, and on exceeding this 15 thickness the deposits invariably become brittle and badly pitted and are worthless. Hence galvanoplasty in nickel and other members of this group of metals has hitherto been impossible.

20 All of the phenomena which cause these difficulties are not known, but it is generally accepted that they are due to the formation of hydrogen or of hydrates of the metals being deposited, according to the conditions 25 of the bath, and the absorption of said hydrogen or hydrate by the metal deposited. The effects of the presence of these absorbed compounds in deposits of nickel, iron, cobalt and their mixtures and alloys are very 30 similar, but as they are more definite and more familiar in the case of nickel deposits, that metal has been selected herein as typical of the group.

In operating baths for the deposition of 35 nickel hydrogen is liberated when the bath is acid and apparently to a slight extent even when it is neutral. On the other hand, when the bath is alkaline the formation of hydrate occurs, and, as the hydrates of 40 nickel and the other members of this group are insoluble, the metal tends to precipitate from the solution and the bath to become inoperative. To avoid this result it is customary in commercial practice to run the 45 baths slightly acid.

Under conditions of commercial operation hydrogen is always present, and forms minute bubbles which adhere with very great tenacity to the cathode. A great many devices have been developed in the operation 60 of baths to remove this hydrogen and to thereby avoid the injurious results which appear to be due to its absorption; for example, heating the cathode, brushing or rolling the cathode, shaking or striking the 65 cathode, adding organic or other materials to the bath, adding solid foreign matter, agitating the bath, etc. These various treatments do not succeed entirely, as with their use the thickness of the deposit may not be 70 appreciably increased above the thickness mentioned, if not actually decreased. The devices employed frequently result in embedding dirt particles in the deposit and thus making it unfit for use, or frequently 75 in causing even greater absorption of hydrogen.

My invention has for its object to render possible the production of deposits of greater thickness than hitherto, to effect the 80 production of deposits that are malleable regardless of their thickness, to render the formation of deposits to a considerable extent independent of the conditions of operation and the amount of impurities and 85 foreign matter in the bath, and such other objects as will hereinafter more fully appear.

I have discovered that the film of hydrogen bubbles which forms upon and adheres so tenaciously to the cathode during the formation of the deposit thereon may be destroyed almost instantaneously by complete removal of the cathode from the bath and exposure thereof to the air. The bubbles of hydrogen, both large and small, seem to burst or disappear almost immediately on removal and the hydrogen contained therein is thus completely removed 90 from the bath. On reimmersing the cathode 95 in the bath any remaining hydrogen film and adhering particles of impurities, such as nickel oxide, in the case of nickel deposition, or other solid impurities, are washed from the cathode by the action of the surface of the solution.

Removal of the metallized cathode from 100 nickel baths or interruption of the current 105 during deposition has hitherto been regarded as to be avoided, as such steps ordinarily 110

cause the deposit forming after reimmersion to have the character of a separate deposit, and to separate or peel away from the deposit below it. I have discovered, however, 5 that if the period of removal from the bath be sufficiently short the subsequently formed deposit forms a homogeneous and integral part of that formed prior to removal, and the entire deposit is unitary and inseparable. 10 I have found that by repeated removal and reimmersion of the cathode from the bath during the deposition process the deposit produced is homogeneous and malleable and may be carried to great thickness, and 15 the bath may be operated under conditions of acidity or alkalinity or impurity which would make deposition otherwise practically impossible, yet without appreciably affecting the malleability and purity of the deposit. 20 Whether this new result is due to complete elimination of hydrogen or whether other factors, such as occlusion of air or oxygen, formation of oxy-compounds in the bath, etc., enter, I have not yet been able to fully 25 determine. Nevertheless this action results in bringing the surface of the deposit into intermittent contact with the gaseous medium, which, as in the case of air, in the example here given, may be of an oxidizing 30 character. This intermittent exposure of the surfaces of the successive deposits to the gaseous medium as by the interposition of a gaseous layer between the surface of each deposit and the liquid of the bath, in 35 the example here given, results in substantially complete dissipation and elimination of hydrogen from the successive layers of the deposited metal, with the consequent production of an electrodeposited metal, such as 40 nickel, in a malleable form.

I have found that the length of the period of removal of the cathode from the bath must be within fairly definite limits in order that the deposit formed after reimmersion 45 may be integral with that formed prior to removal. This critical limit varies with the character of the bath, the temperature of the bath, the difference between the temperature of the bath and the temperature of the air, 50 etc., and may readily be determined by experiment. Thus, in a nickel depositing bath operating 130° F., I have found that the cathode may be removed from the bath for ten seconds without destroying the integral 55 character of the entire deposit, while a removal of fifteen seconds may cause the metal subsequently deposited to form as a distinct, separable layer. With the bath hereinafter 60 specifically described I have found from two to six seconds to be the proper limits of the period of removal when operating at a temperature of 130° F. In any case I find it advisable that the period of removal from the bath be at least two seconds.

65 The frequency of removal is also of im-

portance in connection with the application of my process. I have found that the frequency of removal also depends upon certain factors of the deposition process, particularly the acidity of the bath and the current density; that is, upon those factors which affect the rate of formation of hydrogen in the bath. Thus, the greater the acidity the greater the frequency of removal necessary. In a suitable nickel bath, such 70 as that hereinafter described, with a current density of 200 amperes per square foot, if the bath is very acid, a removal every half minute is necessary; if the bath is only slightly acid, as is the standard practice, a removal every minute or every two minutes is sufficient, and if the bath is perfectly neutral, or even slightly alkaline, removal every five or even ten minutes is sufficient.

In removing the cathode from the bath the current may or may not be shut off during or before removal, as desired. In the case of small cathodes in particular it is unnecessary to cut the current off by auxiliary means. When the cathode is very long in 85 the direction of its movement it may be advisable to cut off the current before removing it to avoid the formation of a deposit thicker at the bottom than at the top. For this purpose any form of circuit breaker may 90 be used, the circuit being open for not more than fifteen seconds and the removal and return of the cathode taking place during this period. When the current is not broken by auxiliary means it may be found desirable 100 to partially rotate the cathode at intervals, preferably while removed from the bath, thereby bringing new points of the cathode to the lowermost position in the bath.

The rate of removal and reimmersion of 105 the cathode may be relatively rapid or slow; I find it desirable, however, to effect them at a relatively rapid rate, thereby diminishing the tendency toward lack of uniformity of the thickness.

It is obvious that the removal and reimmersion of the cathode in the bath may be effected by a great variety of mechanical means. For example, it may be vertically reciprocated into and out of the bath, or it may be mounted on a rotating wheel or arm or moving belt within the bath, a small part of the path of which is outside of the bath. I have illustrated in the accompanying drawing, in part diagrammatically, forms of apparatus such as may be utilized to carry 110 out my process. In the drawing

Figs. 1 and 2 are sections at right angles through a bath in which the cathode is reciprocated vertically into and out of the 115 bath, Fig. 2 being on line 2-2 of Fig. 1.

Figs. 3 and 4 are sections at right angles through a bath in which the cathode is moved through a circular path into and out 120 of the bath.

Referring to the device shown in Figs. 1 and 2, 10 is the vessel containing the bath in which is suspended anode 11 by means of conductor rod 12. The cathode 13, a conductor or non-conductor having its surface graphitized or otherwise made conductive and upon which the metallic deposit is to be formed, is suspended in the bath by means of two arms 14, each having a conductor core 15 conductively attached to the cathode, and surrounded by insulation 16, such as bakelite, hard rubber, or the like. The conductive cores 15 of supporting arms 14 are attached to terminals 17, to which the leads 18, 18 are likewise attached. Terminals 17 are mounted in bar 19, which is slidably mounted on uprights 20 supported by the tank 10 or by any other suitable means. From the rear of bar 19 projects pin 21, which enters the elongated eye 22 of lever 23, which is fulcrumed at 24 on a suitable support. The opposite end 25 of lever 23 projects somewhat into the path of movement of arm 26, which is fixed to shaft 27, mounted on a suitable support and rotated slowly by a pulley or other suitable means 28. The rotation of the arm 26 in the direction indicated by the arrow causes it to engage the end 25 of lever 23 during a small angle of its movement, which may be determined in accordance with the relative periods of immersion and removal of the cathode which, in turn, are determined according to the conditions of operation of the bath, as previously described. The engagement of arm 26 with lever 23 raises the bar 19 and with it the cathode 13 above the surface of the bath (shown in dotted lines) and retains it thereabove until said engagement ceases, at which moment the bar, with the cathode, drops. The forcible reimmersion of the cathode in the bath has a washing action upon the former.

In the device shown in Figs. 3 and 4, 31 is the vessel containing the bath in which the anode 32 is suspended from bar 33. The cathode 34, upon which the deposit is to be formed, is attached to arms 35, which are formed with a conductive core 36, preferably of metal, surrounded by insulating material 37, such as bakelite, the core being conductively connected with the conductive surface of the cathode. The arms 35 are fixed to shaft 38, which is also formed with a conductive core 39 covered by insulating material 40, such as bakelite. The cores 36 of the arm 35 are conductively connected to the core 39 of shaft 38, which core 39 is connected to lead 41. Shaft 38 is passed through stuffing boxes 42 in the sides of the tank, and is rotated by a pulley 43 or other suitable means. The position of the shaft 38 and the length of the arms 35 is such that a small arc of its path is outside the surface of the bath, the angle of this arc and the

rate of movement of the shaft being so selected that the periods and frequency of removal of the cathode are those determined as proper for the conditions of operation of the specific bath in use.

It is obvious that many other mechanical devices may be employed for effecting the periodic removal and reimmersion of the cathode, such as devices of the rotating wheel or moving belt type with a plurality of cathodes attached to the periphery of the wheel or belt, or devices wherein the cathode is maintained stationary and the bath moved toward and away from it. When found advantageous one or more anodes may be placed on each side of the cathode support.

As illustrative of the results which I have obtained, using a bath of the composition:

Nickel sulfate, 240 g.; nickel chloride, 20 g.; boric acid, 40 g.; water, 1 liter, operating at 130° F. and with a current density of 200 amperes per square foot, by removing the cathode for periods of two to six seconds at intervals of one to two minutes, I have formed deposits upwards of one sixteenth of an inch thick and entirely malleable homogeneous and without pits or marks. Under the same conditions without periodic removal of the cathode from the bath, a deposit as thick as 0.004 inch could not be produced without brittleness and excessive pit formation. I have also secured clear malleable deposits of greater thickness than could hitherto be obtained with any bath by means of a bath containing only nickel sulfate and a little sulfuric acid. The character of the result of the process I have found to be the same in the deposition of cobalt, iron and alloys or mixtures of cobalt with nickel etc.

I have furthermore found that the use of my invention prevents to a great degree the deleterious effects of impurities such as iron, copper, arsenic, etc., in the salts of the bath or in the anode, and of solid matter in the bath.

I claim as my invention:

1. In the process of electrodepositing metals, repeatedly removing the cathode surface from the bath for a period of time sufficient to permit the hydrogen on the deposited metal to be substantially eliminated from each successive layer of the deposited metal, and returning it thereto during deposition.

2. In the process of electrodepositing metals, periodically removing the cathode surface from the bath for a period of time sufficient to permit the hydrogen on the deposited metal to be substantially eliminated from each successive layer of the deposited metal, and returning it thereto during deposition.

3. In the process of electrodepositing metals, repeatedly removing cathode surface from the bath and returning it there-

- to during deposition, the period of removal of the cathode surface being less than the critical period at which a separable deposit is formed.
5. 4. In the process of electrodepositing nickel, repeatedly removing the cathode surface from the bath for a period of time sufficient to permit the hydrogen on the deposited metal to be substantially eliminated from each successive layer of the deposited metal, and returning it thereto during deposition.
10. 5. In the process of electrodepositing nickel, periodically removing the cathode surface from the bath for a period of time sufficient to permit the hydrogen on the deposited metal to be substantially eliminated from each successive layer of the deposited metal, and returning it thereto during deposition.
15. 6. In the process of electrodepositing nickel, repeatedly removing the cathode from the bath and returning it thereto during deposition, the period of removal of the cathode being less than the critical period at which a separable deposit of nickel is formed.
20. 7. In the process of electrodepositing nickel, repeatedly removing the cathode from the bath and returning it thereto during deposition, the period of removal of the cathode being not greater than fifteen seconds.
25. 8. In the process of electrodepositing nickel, repeatedly removing the cathode from the bath and returning it thereto during deposition, the period of removal of the cathode being at least two seconds and less than the critical period at which a separable deposit is formed.
30. 9. In the process of electrodepositing metals, repeatedly removing the cathode from the bath and returning it thereto during deposition, the frequency of removal of the cathode varying in accordance with the rate of formation of hydrogen in the bath.
35. 10. In the process of electrodepositing nickel, repeatedly removing the cathode from the bath and returning it thereto during deposition, the frequency of removal of the cathode varying in accordance with the rate of formation of hydrogen in the bath.
40. 11. In the process of depositing nickel by means of a current of high density, removing the cathode at intervals of one half to fifteen seconds for periods of one to fifteen seconds.
45. 12. In the process of electrodepositing metals of the iron group, repeatedly interposing a gaseous medium between the cathode surface and the bath and restoring contact between said surface and said bath, the period of the interposition of the gaseous medium between said surface and said bath being less than the critical period at which a separable deposit is formed.
50. 13. In the process of electrodepositing metals of the iron group, repeatedly interposing a gaseous oxidizing medium between the cathode surface and the bath and restoring contact between said surface and said bath, the period of the interposition of said medium between said surface and said bath being less than the critical period at which a separable deposit is formed.
55. 14. In the process of electrodepositing metals of the iron group, repeatedly interposing air between the cathode surface and the bath and restoring contact between said surface and said bath, the period of the interposition of the air between said surface and said bath being less than the critical period at which a separable deposit is formed.
60. 15. In the process of electrodepositing metals, repeatedly removing cathode surface from the bath and returning it thereto during deposition, the period of removal of the cathode surface being sufficiently great to permit substantially all of the hydrogen on the deposit to be dissipated but less than the critical period at which a separable deposit is formed.
65. 16. In the process of electrodepositing nickel, repeatedly removing cathode surface from the bath and returning it thereto during deposition, the period of removal of the cathode surface being sufficiently great to permit substantially all of the hydrogen in the deposit to be dissipated but less than the critical period at which a separable deposit of nickel is formed.
70. 17. In the process of electrodepositing metals of the iron group, repeatedly removing cathode surface from the bath and returning it thereto during deposition, the period of removal of the cathode surface being sufficiently great to permit substantially all of the hydrogen on the deposit to be dissipated but less than the critical period at which a separable deposit is formed.

CHARLES P. MADSEN.